

## UNITED STATES PATENT OFFICE.

GEORGE H. CHARLS, OF CANTON, OHIO, ASSIGNOR TO UNITED ALLOY STEEL CORPORATION, OF CANTON, OHIO, A CORPORATION OF NEW YORK.

## RESISTANT-SURFACE ALLOY OF IRON.

No Drawing.

Application filed April 14, 1924. Serial No. 706,564.

To all whom it may concern:

Be it known that I, GEORGE H. CHARLS, a citizen of the United States, and a resident of Canton, Stark County, State of Ohio, have invented an Improvement in Resistant-Surface Alloys of Iron, of which the following is a specification.

This invention relates to alloys of iron. One of the objects thereof is to provide a practical iron alloy, the surface of which is thoroughly resistant under conditions of use to any agent tending to corrode or discolor it. Another object is to provide an alloy of the above nature of good physical properties. Another object is to provide an alloy of the above nature which will be inexpensive and suitable for manufacture on a large scale. Other objects will be in part obvious and in part pointed out hereinafter. 20 The invention accordingly consists in the combinations of elements and in the ideas hereinafter illustratively set forth, and the scope of the application of which will be pointed out in the appended claims.

25 Before considering the invention in detail, it may be noted that the term "iron" is used in a broad sense to comprehend not only pure iron but iron including carbon, the latter making what might be more specifically 30 termed "steel". It is also to be noted that the term "resistant surface" is intended to denote a characteristic by virtue of which the entire body of the alloy is such that if its surface be exposed, such surface will resist any agency tending to alter its character, whether by corrosion, staining, heat or otherwise.

In the alloy embodying my invention I include chromium, molybdenum and copper. 40 A composition which I have found to give excellent results comprises copper from .40% to .60%, molybdenum from .05% to .12% and chromium from 16.0% to 20.0%.

The carbon is preferably kept low, by 45 which is meant in this connection .20% or less. An amount of carbon which has given very desirable results is from .03% to .07%.

It is to be understood that none of the above ranges are unnecessary to attain many 50 of the advantages of my invention, as they may be considerably broadened. However, both the copper and molybdenum are preferably to be used in small amounts, as small quantities of them are most efficacious in 55 attaining the desired character of the sur-

face of the alloy. It may be noted that the conjoint use of copper and molybdenum is highly advantageous, as when used together they have an effect markedly superior to that of either used without the other. 60

It is to be understood that in this alloy there are usually present small amounts of phosphorous, sulphur, and other elements commonly present in commercial iron and steel, but such elements are to be kept as 65 low as possible.

I also prefer to add vanadium in an amount ranging from .10% to .50% for best results in scavenging the metal.

The various elements are added preferably with the iron in molten form in such manner as to attain the various constituents throughout the mass of the alloy. 70

As the illustrative alloy above set forth might be varied in many respects without departing from the scope of this invention, it is to be understood that all matters herein set forth are to be interpreted as illustrative and not in a limiting sense. 75

I claim as my invention:— 80

1. A resistant-surface alloy of iron comprising, in combination with the iron, chromium from 3.0% to 30.0%, copper from .10% to 2.0%, and molybdenum from .05% to .35%. 85

2. A resistant-surface alloy of iron comprising, in combination with the iron, carbon in an amount not exceeding .20%, chromium from 3.0% to 30.0%, copper from .10% to 2.0%, and molybdenum from .05% to .35%. 90

3. A resistant-surface alloy of iron comprising, in combination with the iron, carbon in an amount not exceeding .20%, copper from .15% to 2.00%, molybdenum from .05% to .20%, and chromium from 3.0% to 25.0%. 95

4. A resistant-surface alloy of iron comprising, in combination with the iron, carbon in an amount not exceeding .20%, copper from .15% to 2.00%, molybdenum from .05% to .20%, and chromium from 16.0% to 25.0%. 100

5. A resistant-surface alloy of iron comprising, in combination with the iron, carbon in an amount not exceeding .10%, copper from .15% to 2.00%, molybdenum from .05% to .20%, and chromium from 3.0% to 25.0%. 105

6. A resistant-surface alloy of iron com- 110

prising, in combination with the iron, carbon in an amount not exceeding .10%, copper from .20% to .75%, molybdenum from .05% to .20%, and chromium from 16.0% to 25.0%.

7. A resistant-surface alloy of iron comprising, in combination with the iron, carbon in an amount not exceeding .10%, copper from .20% to .75%, molybdenum from .05% to .20%, and chromium from 16.0% to 20.0%.

8. A resistant-surface alloy of iron comprising, in combination with the iron, carbon from .03% to .07%, copper from .20% to .75%, molybdenum from .05% to .20%, and chromium from 16.0% to 25.0%.

9. A resistant-surface alloy of iron comprising, in combination with the iron, carbon from .03% to .07%, copper from .40%

to .60%, molybdenum from .05% to .12%, 20 and chromium from 16.0% to 20.0%.

10. A resistant-surface alloy of iron comprising, in combination with the iron, chromium from 3.0% to 30.0%, copper from .10% to 2.0%, molybdenum from .05% to .35%, and an appreciable amount of vanadium not to exceed .50%.

11. A resistant-surface alloy of iron comprising, in combination with the iron, chromium from 3.0% to 30.0%, copper from .10% to 2.0%, molybdenum from .05% to .35%, carbon in an amount not exceeding .20%, and an appreciable amount of vanadium not exceeding .50%.

In testimony whereof, I have signed my 35 name to this specification this third day of April, 1924.

GEORGE H. CHARLS.